

## UNITED STATES PATENT OFFICE

2,042,393

## COLORED CELLULOSE MATERIAL

Henry Dosne, Mulhouse, France

No Drawing. Original application July 17, 1933,  
Serial No. 680,897. Divided and this applica-  
tion April 30, 1934, Serial No. 723,276. In Ger-  
many August 19, 1932

## 4 Claims. (Cl. 18—54)

This application is divisional of my applica-  
tion Ser. No. 680,897, filed July 17, 1933.

In the said U. S. Patent application Ser. No. 680,897 there is described a process for direct pro-  
duction of dyed regenerated cellulose material  
(viscose) consisting in incorporating into the  
viscous mass in any phase previous to coagulation  
the solution of an ester-salt of a leuco vat dye-  
stuff, in performing the coagulation and finally  
in developing the dyeing in the regenerated cel-  
lulose material by acid oxidation.

As described in said application Serial No. 680,897 this process allows also the production of  
special dyeing effects.

15 It has now been found that in the same way  
also copper silk, obtained by dissolving cellulose  
by means of a solution of ammoniacal copper  
oxide and coagulating the solution with the aid of  
water or diluted acids or alkalies, whereby cel-  
lulose is re-formed, may be directly dyed. Ac-  
20 cording to the present invention a solution of an  
ester-salt of leuco vat dyestuff is added to the  
ammoniacal copper oxide cellulose solution as a  
rule again in any phase of the process previous  
25 to coagulation.

Like in the case of viscose, a completely  
homogeneous mass is thus obtained, in which no  
precipitations or decompositions take place, which  
might adversely affect the subsequent spinning  
30 process and further operations. This mass is then  
spun in the ordinary way and brought to coagulation.  
The produced threads or materials are then  
subjected to the usual after-treatment for  
copper silk.

35 Development of the dyeing takes place by  
means of acid oxidation during coagulation, or by  
a suitable after-treatment of the regenerated  
cellulose after coagulation. As cupric salts in the  
presence of an acid may act as oxidizing agents,  
40 in many cases the copper salt, i. e. the cupric  
sulphate formed in the coagulation bath is suf-  
ficient to develop the dyeing (see U. S. Patent No.  
1,917,101). In this case a further oxidative acid  
treatment is superfluous.

45 The same effects as in the case of viscose may  
generally also be attained with copper silk.

According to the present process it is also pos-  
sible to apply on any kind of fabric an am-  
moniacal copperoxide cellulose mass to which an  
50 ester-salt has been added, to bring the mass to  
coagulation, and to develop the dyeing therein by  
means of acid oxidation during or after coagula-  
tion. In such a way particular effects are ob-  
tained, for example delustrated or shiny relief ef-  
fects, which are dyed fast.

The invention is illustrated, but not limited by  
the following examples:

## Example 1

1 gr. of the ester-salt of leuco diamethoxyli-  
benzanthrone is dissolved in 50 ccm. of lukewarm  
water and 20 ccm. of ammonia of 25%. 20 ccm.  
of this solution are thoroughly mixed with 20  
ccm. of an ammoniacal copper oxide cellulose  
solution. This mixture is spun and coagulated 5  
at 30° C. in a bath containing 40% of sulphuric  
acid. The cellulose is regenerated. The copper  
sulphate formed in the acid coagulation bath acts  
as oxidizing agent and the green dyeing is de-  
veloped during the coagulation process. The thus 10  
obtained threads are subjected to the usual after-  
treatment for copper silk.

## Example 2

1 gr. of the ester-salt of leuco dibenzpyrenequi-  
none is dissolved in 50 ccm. of hot water. After  
cooling down, 20 ccm. of ammonia of 25% are  
added. 20 ccm. of this solution are thoroughly  
mixed with 20 ccm. of a concentrated ammoniacal  
copper oxide cellulose solution. The homogene-  
ous mass is spun as usual and the threads are  
coagulated at 40° C. in a bath containing 30% of  
caustic soda lye and if necessary small quantities  
of sugar, glucose, glycerine or any other suitable  
ingredients. The threads are thoroughly rinsed  
in water containing 20 grs. of sulphuric acid of  
66° Bé. per litre. The ester-salt is not dissolved  
away from the fibre, neither in this stage nor in  
the following coagulation bath. Finally the dye-  
ing is developed by treating the material in a bath  
containing 36 grs. of sulphuric acid of 66° Bé., 3  
grs. of sodium nitrite, also 10 grs. of a solution  
of ammonium vanadate 1:1000 per litre at a tem-  
perature of 20—40° C., or in a bath containing 0.5  
gr. of sodium bichromate or potassium bi-  
chromate, 36 grs. of sulphuric acid of 66° Bé., 20  
grs. of a solution of ammonium vanadate 1:1000  
and 2 grs. of oxalic acid per litre. Thus one ob-  
tains artificial silk threads of a bright, fast yel-  
low.

What I claim is:—

1. A process for manufacturing colored cel-  
lulose material, which consists in adding to an  
ammoniacal copperoxide cellulose solution in any  
phase previous to coagulation a solution of an 50  
ester-salt of a leuco vat dyestuff, performing the  
coagulation in known manner and developing the  
dyeing in the regenerated cellulose by acid oxida-  
tion.

2. A process for manufacturing colored cel- 55

lulose material, which consists in adding to an ammoniacal copperoxide cellulose solution an ester-salt of a leuco vat dyestuff, performing the coagulation in a known manner and developing the dyeing in the regenerated cellulose by treating the latter in a bath containing bichromate and acid.

3. A process for manufacturing colored cellulose material, which consists in adding to an ammoniacal copperoxide cellulose solution previous to coagulation a solution of an ester-salt of a leuco vat dyestuff, performing coagulation of the mass by pressing same into a bath contain-

ing sulphuric acid, whereby owing to the formation of coppersulphate acting in presence of acid as oxidizing agent, simultaneously with the coagulation the development of the dyeing in the regenerated cellulose takes place.

5

4. The herein described colored cellulose material obtained by adding to an ammoniacal copperoxide cellulose solution a solution of an ester-salt of a leuco vat dyestuff, performing coagulation in a known manner and developing the dyeing in the regenerated cellulose by acid oxidation.

10

HENRY DOSNE.